

# UNITED STATES PATENT OFFICE.

PIERRE DRONIER, OF PARIS, FRANCE.

## PROCESS OF MAKING BRONZE ALLOYS.

SPECIFICATION forming part of Letters Patent No. 267,742, dated November 21, 1882.

Application filed April 16, 1881. (Specimens.) Patented in France December 5, 1878, No. 127,801.

*To all whom it may concern:*

Be it known that I, PIERRE DRONIER, of the city of Paris, and Republic of France, have invented a new and useful Improvement in the 5 Process of Making Bronze Alloys, of which the following is a specification.

This invention has for its object the formation of malleable compounds of bronze alloys of copper and tin.

10 In carrying out my invention I employ an intermediate or uniting body. This substance is mercury. I have discovered that mercury introduced in very small quantities in any of the alloys to which I have referred so changes 15 the conditions of these bodies as to render them malleable like copper and similar substances. The proportion of mercury used may be varied according to the different proportions of the alloys. It may be varied from one-half per 20 cent. to two per cent. I have discovered the fact that it is not absolutely necessary that the mercury form part of the new alloys. Its office seems to be catalytic, or more mechanical than chemical. I am of the opinion that this 25 very subtle body, while it passes into the condition of vaporata relatively low temperature, being expanded in the body of the alloy compounds opens the pores of the metallic compounds and thereby favors the penetration of 30 the tin into the copper—in a word, occasions a more intimate mingling between the two metals—perhaps a complete mingling.

In effecting the amalgamation of the bronze alloy I have obtained very good results by 35 mingling the mercury with molten tin in the proportion of one per cent. or two per cent. and adding this mixture to the molten copper. The mercury thus introduced during the process of mixing the molten metals is to a great 40 extent lost, so that the subsequent analysis of

the alloy does not show this substance as one of the constituents thereof. Whichever way the mercury is used the bronze formed with the added mercury will be found to be entirely malleable. It is possible to wire-draw it, roll 45 it, stamp it, and strike it up, and indeed to work it in the same manner as malleable metals. This bronze is harder, more elastic, and more sonorous than the kinds previously made. It is also admirably adapted to the making of 50 musical instruments, and will also be readily employed in the making of apparatus for sugar factories, refineries, and many other industrial operations. Indeed it may be said that the new metal may replace copper in many 55 industrial processes.

I am aware that alloys have been made of copper, tin, and mercury, and I do not claim the combination of these metals, my invention being distinguished from what has preceded it 60 by the fact that I secure a true bronze of copper and tin, using mercury only as a means to this end and securing a product having the desired qualities, yet without retaining the mercury as one of the ingredients of the alloy. 65

What I claim as my invention, and desire to secure by Letters Patent, is—

The within-described process of producing a malleable bronze, the same consisting in mixing mercury with the metals while the same 70 are in a molten state at a temperature to distill the mercury as or after the mixture is effected, whereby a malleable alloy is formed of copper and tin substantially free from mercury, as set forth.

PIERRE DRONIER.

Witnesses:

A. BEQUET,  
MCE. SAUSSERE.